

Dec. 16, 1941.

J. J. BONESTEEL

2,266,155

METALLURGICAL PROCESS

Filed May 31, 1939

2 Sheets-Sheet 1

Ore + Au + X

*Fig. 1.*

$\text{Na}_2\text{CO}_3 + \text{H}_2\text{O}$   
20 lbs. dispersant  
per 1000 gals  $\text{H}_2\text{O}$   
per ton of Ore

Brown to cherry red liquor

Take up in  
Aqua Regia  
Chlorinate or  
Treat with  $\text{NaCN}$

Recover by  
Known Methods



Inventor:  
James J. Bonesteel  
By:-  
Barry V. Wissner  
Atty.

Dec. 16, 1941.

J. J. BONESTEEL

2,266,155

METALLURGICAL PROCESS

Filed May 31, 1939

2 Sheets-Sheet 2

Ore + Au + X

Fig. 2.



Inventor:  
James J. Bonesteel  
By  
Barry V. Wissner  
Atty.

## UNITED STATES PATENT OFFICE

2,266,155

## METALLURGICAL PROCESS

James J. Bonesteel, Chicago, Ill.

Application May 31, 1939, Serial No. 276,671

10 Claims. (CL. 75—118)

This invention concerns itself with the extraction of gold found in finely divided form in sedimentary or argillaceous rocks or like substances. Gold has hitherto been found in such formations in certain localities, certain types of limestone being an example, but fire assay results thereon are very variable, running from a trace to substantial values.

One method of extracting gold from ore of this type is described in copending application of Henry Jeffs and E. J. Dunn, Serial No. 238,646, filed November 3, 1938, to which reference is hereby had for the methods there disclosed. This invention concerns itself with an alternative method for extracting gold from such ores.

It is not known in what state, either physical or chemical, the gold is contained in these ores other than that, in whatever state it may be found, the size of the particles is sub-microscopic, hereinafter referred to for convenience as gold micelle or micellie gold. The actual size of the gold micelle may vary from a few millimicrons for the smallest, up to one micron for the largest. Whether the gold is free or in the form of oxides or salts is not known. It has been found, however, that by the use of certain reagents the gold micelle in the ore can be put into a colloid state in a hydrosol from which the values can readily be extracted by known methods.

The object of this invention, therefore, is to provide means to extract micellie gold from its ores through dispersion into a hydrosol. Two methods of accomplishing this result present themselves, one comprising a direct method of putting the micellie gold from the ore into a hydrosol, and the other comprising an indirect method after concentrating the ore. The direct method is diagrammatically shown in the flow sheet marked Fig. 1 in the drawings; the indirect method is shown in the flow sheet marked Fig. 2.

*Direct method*

The ore is first comminuted as finely as can conveniently be done. Ordinary comminution methods will produce particles capable of passing two to three hundred mesh, a size which has been found adequate for the purpose of the invention, although, it is to be understood, other things being equal, that the finer the comminution the more efficacious the process. Comminution may be either wet or dry, but, if wet methods are used, care should be taken to preserve all the fluid.

After comminution has been completed, the gangue is attacked with a dispersing or peptizing

agent, such as sodium carbonate, in water. In practice half a gallon of water has been used per pound of ore. The proportion of the dispersing or peptizing agent used varies with the particular reagent. In practice, about twenty pounds of sodium carbonate per ton of ore will produce an incipient hydrosol from comminuted limestone within a short time interval, about one half hour.

It is to be understood, however, that the quantity and type of dispersing or peptizing agent will vary with the type of ore treated and the optimum can only be determined after some experiment.

As a dispersing or peptizing agent, sodium carbonate is preferred, although sodium oxalate, sodium hydroxide, ammonium hydroxide and di-glycol laurate have been found useful. Many other dispersing agents are known in the chemical arts, but the permutations of their number and chemical properties make it impossible to disclose their effect in or pertinence to the use in the described process.

After the addition of the dispersing or peptizing agent, the liquor is shaken or agitated, the time interval used in practice being sixteen to forty-eight hours. During the agitation interval, the gold micelle in the ore will be dispersed by the dispersing or peptizing agent into a colloid state, in a liquor characterized by typical colloid colors. Sodium carbonate will produce a hydrosol characterized by a brown or cherry red color within a short time interval. As its action continues, the color of the liquor will deepen until in from twenty-four to forty-eight hours, it becomes an intense brown or red. At this point, the agitation and dispersion step is completed.

It has been found that a very much longer time interval will produce a liquor having a black color to reflected light. If the liquor is permitted to stand, even without agitation, for a period of from ninety to one hundred twenty days, dispersion of the micelle from the gangue will continue with the eventual result of such a black color.

After the agitation and dispersion step, the liquor is filtered through a paper filter, and the gangue is washed in water through the filter until the water coming through is free from color. The gangue remaining may be considered as tailings, although it is ordinarily good practice to redisperse or peptize the gangue and pass it through the agitation and filter stages, as previously described, until no further hydrosols can be established through the dispersion and agitation.

The filtrate, as pointed out, may vary from a

brown to a black color in reflected light. The gold can be extracted from the filtrate through dissolution by known methods, as chlorination, aqua regia or sodium cyanide, for example.

Alternately, the gold may be extracted from the filtrate through coagulation, comprising the addition of a coagulant such as, for example, acetic or a mineral acid in an amount sufficient to make the solution distinctly acid to litmus. After addition of the coagulant, the liquor should be heated until flocculation occurs. The coagulated liquor is then filtered through a treated paper filter or an extremely fine porcelain filter, the values being recovered after filtration by known methods.

#### *Indirect method*

The indirect method, diagrammatically shown in Fig. 2 of the drawings, comprises first concentrating the ore after it has been comminuted as previously described.

After comminution, the ore is first treated with a six per cent. solution of hydrogen peroxide in the amount of one half gallon of solution per pound of ore, the time interval for the reaction continuing until all action ceases, probably sixteen to twenty-four hours, the result being a fluid and slime.

The product is then treated with concentrated hydrochloric acid in amount sufficient to complete the reaction, leaving the solution still slightly acid, after which the product comprises a mixture of fluid slime and scum, the mass of slime being approximately one-tenth of the original aggregate.

The product is then filtered without dilution through a filter paper, the residue being washed with water in an amount sufficient to free it from any remaining hydrochloric acid.

The residue is then removed from the filter paper and treated with a dispersing or peptizing agent, the preferred agent being a five per cent. solution of di-glycol laurate, although sodium carbonate, sodium and ammonium hydroxides, or sodium oxalate may be used. The amount of di-glycol laurate used is about one gallon to five quarts per pound of concentrate. The liquor is then shaken or agitated for a time interval, sixteen hours having been found adequate in practice, during the course of which it will acquire a deep cherry red color.

The liquor is then filtered through a filter paper and the residue washed in water until no more color comes through, after which the gold may be captured from the liquor through dissolution by chlorination or aqua regia, or by coagulation and further filtration as previously described.

"Micelle" is herein defined to cover minute particles having a diameter from a few millimicrons up to one micron, lacking appreciable mass.

It is to be understood that the foregoing description is illustrative only and may be departed from, in so far as the resort to equivalents is concerned, without a departure from the spirit of the invention.

Having fully described the invention, I claim:

1. In the art of extracting gold micelle from

its ores, that process which comprises comminution of the ore, dispersion of the gold or its compounds by physico-chemical means from the ore into a colloid state, filtration from the gangue of the liquor resulting from dispersion, and recovery of the gold from the filtrate.

2. In the art of extracting gold micelle from its ores, that process which comprises comminuting the ore, dispersing the gold or its compounds therein by physico-chemical means into a hydrosol, having a characteristic gold colloid color, filtration of the hydrosol from the gangue, and recovery of the gold from the hydrosol.

3. In the art of recovering gold micelle from the natural state, those steps in the process comprising attacking treated ore containing the micelle with a gold-selective dispersing or peptizing agent and agitating the liquor until a gold hydrosol is formed.

4. In the art of extracting gold micelle from its ores, that process which comprises comminution of the ore, concentration of the ore through the reaction of solvents therefor, treatment of the concentrate with a gold-selective dispersing or peptizing agent, the formation of a gold hydrosol, having a characteristic gold colloid color, and the recovery of the gold from the hydrosol.

5. In the art of extracting gold micelle from its ores after the same have been concentrated through the reaction of solvents, that step which comprises attacking the concentrate with a gold-selective dispersing or peptizing agent.

6. In the art of recovering gold micelle from the natural state, those steps in the process comprising attacking concentrated ore containing the micelle with a gold-selective dispersing or peptizing agent and agitating the liquor until a gold hydrosol, having a characteristic gold colloid color, is formed.

7. In the art of recovering gold micelle from the natural state, those steps in the process comprising attacking comminuted ore containing the micelle with a gold-selective dispersing or peptizing agent and agitating the liquor until a gold hydrosol, having a characteristic gold colloid color, is formed.

8. In the art of recovering gold micelle from the natural state, those steps in the process comprising attacking treated ore containing the micelle with a gold-selective dispersing or peptizing agent and permitting the liquor to stand until a gold hydrosol, having a characteristic gold colloid color, is formed.

9. In the art of recovering gold micelle from the natural state, those steps in the process comprising attacking concentrated ore containing the micelle with a gold-selective dispersing or peptizing agent and permitting the liquor to stand until a gold hydrosol, having a characteristic gold colloid color, is formed.

10. In the art of recovering gold micelle from the natural state, those steps in the process comprising attacking comminuted ore containing the micelle with a gold-selective dispersing or peptizing agent and permitting the liquor to stand until a gold hydrosol, having a characteristic gold colloid color, is formed.

JAMES J. BONESTEEL.